

# UNITED STATES PATENT OFFICE.

CHARLES E. GRIFFING, OF LOS ANGELES, CALIFORNIA, ASSIGNOR TO WILLIAM H. KENNEDY, OF LOS ANGELES, CALIFORNIA.

## EXPLOSIVE.

1,282,413.

Specification of Letters Patent. Patented Oct. 22, 1918.

No Drawing. Application filed May 31, 1917, Serial No. 171,877. Renewed March 18, 1918. Serial No. 293,250.

To all whom it may concern:

Be it known that I, CHARLES E. GRIFFING, a citizen of the United States, residing at Los Angeles, in the county of Los Angeles, State of California, have invented new and useful Improvements in Explosives, of which the following is a specification.

This invention relates to explosives and particularly to gun powder; and it is an object of this invention to provide a gun powder of high efficiency which may be easily and cheaply manufactured without special or expensive machinery, without danger of explosion, and which will retain its strength for long periods of time. I accomplish these objects by making the following described mixture in the following described manner.

I take first 49% of white granulated sugar and dissolve it in sufficient water, boiling the solution until it forms a syrup which will harden when cooled. This is then removed from the heat and powdered chlorate of potassium 50% is stirred into it. The mass is stirred until it is of the consistency of soft putty and is then granulated by being rubbed through a screen with meshes the size of the grains desired in the finished powder. When this granulated mass is thoroughly dried, it is mixed with the following dry powdered ingredients: permanganate of potassium  $\frac{1}{2}$  of 1%, powdered white sulfur  $\frac{1}{2}$

of 1%, talcum powder  $\frac{1}{2}$  of 1%; the talcum powder lubricating and smoothing the grains.

This explosive is particularly suitable as a gun powder, being of great strength and being smokeless.

Having described a preferred form of my invention, I claim:

1. An explosive consisting of a granulated mixture of powdered chlorate of potassium 50%, sugar 49%, permanganate of potassium  $\frac{1}{2}$  of 1%, sulfur  $\frac{1}{2}$  of 1% and talcum powder  $\frac{1}{2}$  of 1%.

2. An explosive consisting of a granulated mixture of powdered chlorate of potassium 50%, white granulated sugar 49%, permanganate of potassium  $\frac{1}{2}$  of 1%, powdered white sulfur  $\frac{1}{2}$  of 1%, and talcum powder  $\frac{1}{2}$  of 1%.

3. An explosive comprising chlorate of potash, sugar, permanganate of potassium, sulfur, and talcum powder.

4. An explosive consisting exclusively of chlorate of potash, sugar, permanganate of potassium, sulfur, and talcum powder.

In witness that I claim the foregoing I have hereunto subscribed my name this 24th day of May 1917.

CHARLES E. GRIFFING.

Witness:

JAMES T. BARKELEW.